# EUROPEAN PATENT SPECIFICATION

(11) **EP 4 361 297 B1**
(45) Date of publication and mention of the grant of the patent: **22.07.2026**
(21) Application number: 23207041.7
(22) Date of filing: 31.10.2023
(51) Int. Cl.: C22C 1/02, C22C 19/05, C22F 1/10

(54) **NI-BASED ALLOY AND METHOD FOR MANUFACTURING THE SAME, AND NI-BASED ALLOY MEMBER**
NI-BASIERTE LEGIERUNG UND VERFAHREN ZUR HERSTELLUNG DAVON SOWIE ELEMENT AUS NI-BASIERTER LEGIERUNG
ALLIAGE À BASE DE NI ET SON PROCÉDÉ DE FABRICATION, ET ÉLÉMENT EN ALLIAGE À BASE DE NI

(30) Priority: 31.10.2022 JP 2022174050; 07.08.2023 JP 2023128787
(43) Date of publication of application: 01.05.2024
(73) Proprietor: Daido Steel Co., Ltd., Nagoya-shi Aichi 461-8581 (JP)
(72) Inventor: Furusho, Chihiro, Nagoya-shi, 457-8545 (JP); Koyanagi, Yoshihiko, Nagoya-shi, 457-8545 (JP); Roy, Indranil, Houston, 77099 (US)
(74) Representative: Diehl & Partner

(56) References cited:
- JP-B2- 5 437 669
- US-A1- 2016 215 660
- US-A1- 2021 062 314
- US-B2- 7 682 474
- DEMPSTER IAN ET AL: "Heat Treating of Nonferrous Alloys", 1 June 2016 (2016-06-01), pages 399 - 425, XP093132823, ISBN: 978-1-62708-169-6, Retrieved from the Internet <URL:https://dl.asminternational.org/handbooks/edited-volume/chapter-pdf/517464/a0006261.pdf> DOI: 10.31399/asm.hb.v04e.a0006261

## Description

### TECHNICAL FIELD

The present invention relates to a Ni-based alloy and a method for manufacturing the same, and a Ni-based alloy member, and more particularly, relates to a Ni-based alloy excellent in impact resistance, wear resistance, and corrosion resistance, and a method for manufacturing the same, and a Ni-based alloy member composed of such a Ni-based alloy.

### BACKGROUND ART

Examples of an alloy generally excellent in wear resistance include (a) tool steel (for example, SKD11 (G 4404 : 2015)) and (b) martensitic stainless steel (for example, SUS440C).

However, these Fe-Cr-C alloys are inferior in corrosion resistance, and thus are not suitable for use in environments such as in seawater where corrosion resistance is required.

Examples of an alloy with high corrosion resistance that generally withstands seawater includes (a) austenitic stainless steel (for example, SUS316L(G 4305 : 2012 )), (b) titanium alloys, and (c) nickel alloys (for example, 718 alloy, 625 alloy).

However, these alloys are lower in hardness than tool steels or martensitic stainless steels and significantly inferior in wear resistance to them.

Furthermore, applications of such highly corrosion-resistant alloys with excellent wear resistance include members for oil and gas drilling. Such members are processed from shaped materials, round bars or wires produced by hot forging or hot rolling. Therefore, it is also important for these alloys to have sufficient hot workability for mass production.

In order to solve this problem, various proposals have been made in the related art.

For example, Patent Literature 1 discloses a Ni-based high-strength heat-resistant alloy obtained by manufacturing an ingot containing 0.1 mass% or less of C, predetermined amounts of Si, Mn, Cr, and Al, with the balance being Ni and unavoidable impurities, and then subjecting the ingot to hot forging, solution heat treatment, and aging treatment.

Patent Literature 1 also describes that (A) by such a method, a Ni-based alloy in which y' phase and α phase are compositely precipitated can be obtained, and (B) in addition to the y' phase, composite precipitation of the α phase, which mainly contains Cr, provides a Ni-based alloy with high strength, high-temperature stability, high hardness, high corrosion resistance, and non-magnetism.

Patent Literature 2 discloses a Ni-based alloy obtained by manufacturing an ingot containing more than 0.10 mass% and 1.0 mass% or less of C, predetermined amounts of Cr, Al and V, with the balance being Ni and impurities, and then subjecting the ingot to hot forging, solution heat treatment, and aging treatment.

Patent Literature 2 also describes that (A) in the case where the C content exceeds 0.10 mass%, hard particles (Cr-based carbides containing V) are crystallized in the matrix, resulting in a significant improvement in wear resistance, and (B) when Cr is consumed to form carbides, the amount of Cr dissolved in the matrix decreases, and therefore the precipitation amount of α phase during aging treatment decreases, making it impossible to obtain high hardness, and (C) in the case where V is added to the Ni-based alloy, part of the Cr in the Cr-based carbide is replaced with V, and the amount of Cr consumed to form the carbides is reduced, resulting in high hardness after aging treatment.

As described in Patent Literature 1, the composite precipitation of the γ' phase and the α phase (Cr) can be used to obtain a Ni-based alloy with a Vickers hardness exceeding 600 HV at room temperature. This Ni-based alloy is excellent in hot workability and also has corrosion resistance in a seawater environment. However, this Ni-based alloy does not include a microstructure in which hard coarse carbides are dispersed as the tool steel or the martensitic stainless steel, and therefore, wear resistance thereof is low for hardness thereof.

By using the method described in Patent Literature 2, a Ni-based alloy in which Cr-based carbides containing V are dispersed in the matrix is obtained. This Ni-based alloy is excellent in wear resistance since hard particles are contained therein. In order to prevent a decrease in hardness due to a decrease in dissolved Cr, this Ni-based alloy has a preferable lower limit of the Cr content of 36 mass%, and partially replaces Cr in the Cr carbide with V. However, although such a microstructure contributes to an improvement in hardness, it also causes a decrease in toughness. Especially, since a large impact is applied to a member for oil and gas drilling during drilling, the Ni-based alloy described in Patent Literature 2 is not suitable for a member for oil and gas drilling in terms of an impact property. Patent Literature 3 discloses a cutter composed of a Ni-Cr-Al alloy containing from 32 to 44 mass% of Cr and from 2.3 to 6.0 mass% of Al, the balance being Ni, impurities and trace elements.
Patent Literature 1: JP 4419298 B2
Patent Literature 2: JP 6521418 B2
Patent Literature 3: US 7 682 474 B2

### SUMMARY OF THE INVENTION

The problem to be solved by the present invention is to provide a Ni-based alloy suitable as a material for various members requiring impact resistance, wear resistance, and corrosion resistance, and a method for manufacturing the same.

Another problem to be solved by the present invention is to provide a Ni-based alloy member composed of such a Ni-based alloy.

In order to solve the above-mentioned problems, a Ni-based alloy according to the first embodiment of the present invention consists of: $0.10 mass % < C \leq 0.30 mass % ;$ $Si \leq 0.50 mass % ;$ $Mn \leq 0.50 mass % ;$ $P \leq 0.030 mass % ;$ $S \leq 0.010 mass % ;$ $Cu \leq 3.00 mass % ;$ $30.0 mass % \leq Cr \leq 39.0 mass % ;$ $Mo \leq 3.00 mass % ;$ $Fe \leq 3.00 mass % ;$ $2.00 mass % \leq Al \leq 5.00 mass % ;$ $O \leq 0.0100 mass % ;$ $N \leq 0.050 mass % ;$ $Nb \leq 0.50 mass % ;$ $V \leq 0.50 mass % ;$ $Ti \leq 0.50 mass % ;$ $Ta \leq 0.50 mass % ;$ $W \leq 0.50 mass % ;$ and
at least one element selected from the group consisting of 0.0010 mass% ≤ B ≤ 0.0100 mass%, 0.0010 mass% ≤ Mg ≤ 0.0100 mass%, and 0.0010 mass% ≤ Ca ≤ 0.0100 mass%,
with the balance being Ni and unavoidable impurities, in which
the Ni-based alloy includes
   an austenite phase (y phase) having an average grain diameter of 50.0 µm or less,
   a M₂₃C₆-type carbide having an average circle equivalent particle diameter of 1.0 µm or more, and
   a massive α-Cr phase having an average circle equivalent particle diameter of 10.0 µm or less.

A Ni-based alloy member according to the first embodiment of the present invention is composed of the Ni-based alloy according to the first embodiment of the present invention.

A Ni-based alloy according to the second embodiment of the present invention consists of: $0.10 mass % < C \leq 0.30 mass % ;$ $Si \leq 0.50 mass % ;$ $Mn \leq 0.50 mass % ;$ $P \leq 0.030 mass% ;$ $S \leq 0.010 mass% ;$ $Cu \leq 3.00 mass% ;$ $30.0 mass% \leq Cr \leq 39.0 mass% ;$ $Mo \leq 3.00 mass% ;$ $Fe \leq 3.00 mass% ;$ $2.00 mass% \leq Al \leq 5.0 mass% ;$ $O \leq 0.0100 mass% ;$ $N \leq 0.050 mass% ;$ $Nb \leq 0.50 mass% ;$ $V \leq 0.50 mass % ;$ $Ti \leq 0.50 mass % ;$ $Ta \leq 0.50 mass ;$ $W \leq 0.50 mass % ;$ and
at least one element selected from the group consisting of 0.0010 mass% ≤ B ≤ 0.0100 mass%, 0.0010 mass% ≤ Mg ≤ 0.0100 mass%, and 0.0010 mass% ≤ Ca ≤ 0.0100 mass%,
with the balance being Ni and unavoidable impurities, in which
the Ni-based alloy includes
   a cellular structure,
   a M₂₃C₆-type carbide having an average circle equivalent particle diameter of 1.0 µm or more, and
   a massive α-Cr phase having an average circle equivalent particle diameter of 10.0 µm or less,
in which the cellular structure is a structure in which a lamellar structure of the α-Cr phase and a y phase in which a y' phase is precipitated is formed in a state of cell on an entire inside of an austenite phase,
in which the Ni-based alloy has a 0.2% proof stress at 25°C of 1300 MPa or more, and
in which the Ni-based alloy has an absorption energy at 25°C of 40 J (10 R notch) or more.

A Ni-based alloy member according to the second embodiment of the present invention is composed of the Ni-based alloy according to the second embodiment of the present invention.

A method for manufacturing a Ni-based alloy, the method including:
a first step of obtaining an ingot by melting and casting a raw material blended to have a predetermined composition;
a second step of obtaining a primary hot-worked product by subjecting the ingot to primary hot working;
a third step of obtaining a homogenized heat-treated product by subjecting the primary hot-worked product to homogenization heat treatment;
a fourth step of obtaining a secondary hot-worked product by subjecting the homogenized heat-treated product to secondary hot working; and
a fifth step of obtaining the Ni-based alloy according to the first embodiment of the present invention by subjecting the secondary hot-worked product to solution heat treatment, wherein the solution heat treatment includes holding the secondary hot-worked product at a temperature in the range of 980°C to 1080°C for at least 0.5 to 1 hour.

The method for manufacturing a Ni-based alloy according to the present invention, the method may further include:
a seventh step of obtaining the Ni-based alloy according to the second embodiment of the present invention by subjecting the Ni-based alloy after the solution heat treatment to aging treatment.

In the case where the raw material of the Ni-based alloy containing a relatively large amount of C is melted and cast, an ingot containing the massive α-Cr phase and crystallized coarse M₂₃C₆-type carbide particles can be obtained. If necessary, the obtained ingot is subjected to the primary hot working, homogenization heat treatment, and secondary hot working, and then solution heat treatment at a relatively low temperature, so that a fine massive α-Cr phase remains without being dissolved. As a result, the fine massive α-Cr phase functions as pinning particles, and during the solution heat treatment, coarsening of the y phase can be prevented. Furthermore, when the aging treatment is applied to the Ni-based alloy after the solution heat treatment, the cellular structure is formed on the entire inside of the y phase.

The Ni-based alloy according to the present invention is excellent in corrosion resistance and hot workability due to an optimized composition thereof. The Ni-based alloy after the aging treatment exhibits high wear resistance since the coarse M₂₃C₆-type carbide particles are dispersed in a matrix. Furthermore, the Ni-based alloy after the aging treatment exhibits high strength due to the inclusion of the cellular structure. Since an initial y phase is fine, the cellular structure is also fine, and high toughness (that is, high impact resistance) is also exhibited.

### BRIEF DESCRIPTION OF DRAWINGS

FIG. 1 is an example of a phase map obtained by SEM-EBSD of a Ni-based alloy (Example 4) after solution heat treatment.
FIG. 2 is an example of a phase map obtained by SEM-EBSD of the Ni-based alloy (Example 4) after aging treatment.

### DESCRIPTION OF EMBODIMENTS

Hereinafter, an embodiment of the present invention will be described in detail.

### 1. Ni-based Alloy (1)

### 1.1. Components

The Ni-based alloy according to the first embodiment of the present invention consists of the following elements, with the balance being Ni and unavoidable impurities. Types of additive elements, component ranges thereof, and reasons for limitation thereof are as follows.

### (1) 0.10 mass% < C ≤ 0.30 mass%:

C is an element for forming hard carbides (M₂₃C₆-type carbides) that ensure wear resistance. In the case where an amount of C is too small, an amount of the hard carbide decreases and the wear resistance decreases. In order to obtain a sufficient wear resistance, it is necessary that the amount of C exceeds 0.10 mass%. The amount of C is preferably 0.12 mass% or more, and more preferably 0.14 mass% or more.

On the other hand, in the case where the amount of C becomes excessive, hot workability deteriorates. Therefore, it is necessary that the amount of C is 0.30 mass% or less. The amount of C is preferably 0.28 mass% or less, and more preferably 0.26 mass% or less.

### (2) Si ≤ 0.50 mass%:

Si is an element included as an impurity. Since Si lowers strength and toughness of the Ni-based alloy, the smaller a content thereof, the better. In order to prevent deterioration in the strength and toughness, it is necessary that an amount of Si is 0.50 mass% or less. The amount of Si is preferably 0.10 mass% or less.

### (3) Mn ≤ 0.50 mass%:

Mn is an element included as an impurity. On the other hand, Mn fixes S included in the Ni-based alloy as MnS, and has an effect of preventing deterioration of the hot workability due to S. Therefore, the Ni-based alloy may include Mn.

However, in the case where an amount of S is sufficiently small (for example, in the case where the amount of S is 0.002 mass% or less), it is not necessary to add Mn. The addition of Mn more than necessary may cause deterioration of performance of the Ni-based alloy. Therefore, it is necessary that an amount of Mn is 0.50 mass% or less. The amount of Mn is preferably 0.10 mass% or less.

### (4) P ≤ 0.030 mass%:

P is an element included as an impurity. Since P deteriorates the hot workability, the smaller a content thereof, the better. In order to prevent the deterioration in the hot workability, it is necessary that an amount of P is 0.030 mass% or less. The amount of P is preferably 0.010 mass% or less, and more preferably 0.005 mass% or less.

### (5) S ≤ 0.010 mass%:

S is an element included as an impurity. Since S deteriorates the hot workability, the smaller a content thereof, the better. In order to prevent the deterioration in the hot workability, it is necessary that the amount of S is 0.010 mass% or less. The amount of S is preferably 0.003 mass% or less, and more preferably 0.002 mass% or less.

### (6) Cu ≤ 3.00 mass%:

Cu has an effect of improving corrosion resistance of the Ni-based alloy. Therefore, the Ni-based alloy may include Cu.

However, in the case where an amount of Cu becomes excessive, the hot workability may deteriorate. Therefore, it is necessary that the amount of Cu is 3.00 mass% or less. The amount of Cu is preferably 2.50 mass% or less, and more preferably 2.00 mass% or less.

### (7) 30.0 mass% ≤ Cr ≤ 39.0 mass%:

Cr is an element necessary to ensure the hardness and wear resistance of the Ni-based alloy. In the Ni-based alloy according to the present invention, the hardness is ensured by a lamellar structure of an α phase (Cr) and a y/y' phase. Therefore, it is necessary that an amount of Cr is 30.0 mass% or more. The amount of Cr is preferably 34.0 mass% or more.

On the other hand, in the case where the amount of Cr is excessive, an amount of a massive α-Cr phase with poor deformability becomes excessive, thereby deteriorating the hot workability. Therefore, it is necessary that the amount of Cr is 39.0 mass% or less. The amount of Cr is preferably 38.0 mass% or less.

### (8) Mo ≤ 3.00 mass%:

Mo is an element included as an impurity. A content of Mo as an impurity is usually 0.1 mass% or less. On the other hand, Mo has an effect of improving the corrosion resistance. Therefore, the Ni-based alloy may include Mo.

However, in the case where an amount of Mo becomes excessive, the hot workability may deteriorate. Therefore, it is necessary that the amount of Mo is 3.00 mass% or less. The amount of Mo is preferably 2.50 mass% or less, and more preferably 2.00 mass% or less.

### (9) Fe ≤ 3.00 mass%:

Fe is an element included as an impurity. Since Fe deteriorates the corrosion resistance of the Ni-based alloy, the smaller a content thereof, the better. In order to prevent the deterioration in the corrosion resistance, it is necessary that an amount of Fe is 3.00 mass% or less. The amount of Fe is preferably 1.00 mass% or less.

### (10) 2.00 mass% ≤ Al ≤ 5.00 mass%:

Al is an element necessary for obtaining a high-strength Ni-based alloy by forming Ni₃Al (γ' phase). In order to obtain such an effect, it is necessary that an amount of Al is 2.00 mass% or more. The amount of Al is preferably 3.00 mass% or more.

On the other hand, in the case where the amount of Al becomes excessive, the hot workability may deteriorate. Therefore, it is necessary that the amount of Al is 5.00 mass% or less. The amount of Al is preferably 4.50 mass% or less, and more preferably 4.00 mass% or less.

### (11) O ≤ 0.0100 mass%:

O is an element included as an impurity, and the smaller a content thereof, the better. In order to prevent deterioration in the performance of the Ni-based alloy, it is necessary that an amount of O is 0.0100 mass% or less.

### (12) N ≤ 0.050 mass%:

N is an element included as an impurity, and the smaller a content thereof, the better. In order to prevent deterioration in the performance of the Ni-based alloy, it is necessary that an amount of N is 0.050 mass% or less.
(13) Nb ≤ 0.50 mass%:
(14) V ≤ 0.50 mass%:
(15) Ti ≤ 0.50 mass%:
(16) Ta ≤ 0.50 mass%:
(17) W ≤ 0.50 mass%:

Nb, V, Ti, Ta, and W are all elements included as impurities. These elements combine with C and/or N in the Ni-based alloy to form carbides (MC), nitrides (MN), and/or carbonitrides (M (C, N)) (hereinafter collectively referred to as "MC-type carbonitrides"). Fine MC-type carbonitrides contribute to an improvement in hardness, but cause a deterioration in toughness. In the case where contents of these elements become excessive, C in the Ni-based alloy is consumed to form the MC-type carbonitrides. As a result, formation of a M₂₃C₆-type carbide is inhibited, and the wear resistance deteriorates. Therefore, it is necessary that the content of each of these elements is 0.50 mass% or less. The lower the contents of these elements, the better, and the content of each of these element is preferably 0.40 mass% or less, and more preferably 0.30 mass% or less.
(18) 0.0010 mass% ≤ B ≤ 0.0100 mass%:
(19) 0.0010 mass% ≤ Mg ≤ 0.0100 mass%:
(20) 0.0010 mass% ≤ Ca ≤ 0.0100 mass%:

All of B, Mg and Ca are elements that improve the hot workability. The Ni-based alloy may include only one of B, Mg, and Ca, or may include two or more thereof. Addition of two or more elements thereof is effective for improving the hot workability.

In the case where an amount of B, Mg, or Ca is too small, the hot workability may deteriorate.
Therefore, it is necessary that the amount of each of B, Mg, or Ca is 0.0010 mass% or more.

On the other hand, in the case where the amount of each of B, Mg, or Ca is excessive, hard inclusions containing B, Mg, and/or Ca are formed, and the toughness of the Ni-based alloy may deteriorate. Therefore, it is necessary that the amount of each of B, Mg, or Ca is 0.0100 mass% or less.

### 1.2. Microstructure

### 1.2.1. Austenite Phase

### A. Overview

The Ni-based alloy according to the present embodiment is obtained by
(a) melting and casting a raw material blended to have a predetermined composition,
(b) subjecting an ingot to primary hot working and/or homogenization heat treatment if necessary,
(c) subjecting the ingot, a primary hot-worked product, or a homogenized heat-treated product to secondary hot working, and
(d) subjecting the secondary hot-worked product to solution heat treatment.

Therefore, the Ni-based alloy according to the present embodiment includes a microstructure in which the M₂₃C₆-type carbide and the massive α-Cr phase are dispersed in the austenite phase (y phase). The composition of the y phase is uniquely determined according to the raw material composition, a precipitation amount of the M₂₃C₆-type carbide, and a precipitation amount of the massive α-Cr phase. The y phase becomes a cellular structure by aging treatment. Details of the cellular structure will be described later.

### B. Average Grain Diameter

An "average grain diameter of y phase" refers to a value measured by a line segment method.

The smaller an average grain diameter of the γ phase before the aging treatment, the smaller an average grain diameter of the cellular structure formed by the aging treatment. As the average grain diameter of the cellular structure becomes smaller, the toughness (that is, impact resistance) of the Ni-based alloy after the aging treatment is improved. In order to obtain such an effect, it is necessary that the average grain diameter of the γ phase is 50 µm or less.

### 1.2.2. M₂₃C₆-type Carbide

### A. Overview

The Ni-based alloy according to the present embodiment includes the M₂₃C₆-type carbide. A coarse M₂₃C₆-type carbide contributes to improvement of the wear resistance of the Ni-based alloy. In the present invention, M is mainly Cr, but may contain other elements (for example, Fe, or Mo) depending on manufacturing conditions.
Note that the word "mainly" means that M contains 90 mass% or more of Cr.

Examples of a method for forming the M₂₃C₆-type carbide in the Ni-based alloy include (a) a method of crystallizing carbides during casting, and (b) a method of precipitating carbides during hot working and/or homogenization heat treatment.

In the case where more than 0.1 mass% of C is added to the raw material containing predetermined amounts of Ni, Cr, and Al, the coarse M₂₃C₆-type carbide can be crystallized during casting.

On the other hand, even in the case where the amount of C included in the raw material is 0.1 mass% or less, the M₂₃C₆-type carbide can be precipitated during hot working and/or during homogenization heat treatment. However, the precipitated carbide often has an average particle diameter of less than 1.0 µm. The fine precipitated carbide is poor in the effect of improving the wear resistance.

Therefore, in order to improve the wear resistance, it is preferable to use the crystallized carbide.

### B. Average Circle Equivalent Particle Diameter

A "circle equivalent particle diameter of the M₂₃C₆-type carbide" refers to a diameter of a circle having an area equal to a cross-sectional area of the M₂₃C₆-type carbide when a cross section of the Ni-based alloy is observed with a microscope (SEM-EBSD).

An "average circle equivalent particle diameter of the M₂₃C₆-type carbide" refers to an average value of circle equivalent particle diameters measured for ten freely selected M₂₃C₆-type carbides when the cross section of the Ni-based alloy is observed with a microscope (SEM-EBSD) at a magnification of 1500 times.

The M₂₃C₆-type carbide remains almost as it is even after the aging treatment and contributes to the improvement in the wear resistance of the Ni-based alloy after the aging treatment. The larger the average circle equivalent particle diameter of the M₂₃C₆-type carbide is, the higher the wear resistance is obtained. In order to obtain such an effect, it is necessary that the average circle equivalent particle diameter of the M₂₃C₆-type carbide is 1.0 µm or more. The average circle equivalent particle diameter is preferably 2.0 µm or more, and more preferably 5.0 µm or more.

An upper limit of the average circle equivalent particle diameter of the M₂₃C₆-type carbide is not particularly limited, but in the case where the crystallized carbide is used, the average circle equivalent particle diameter thereof is usually 100 µm or less.

### C. Content

A "content of the M₂₃C₆-type carbide" refers to a value obtained by (a) extracting a test material having a predetermined size from the Ni-based alloy, (b) anodic dissolving a part of the test material for approximately 2 hours to 5 hours at a current density of 25 mA/cm² by constant current electrolysis using a 10 volume% acetylacetone-1 mass% tetramethylammonium chloride-methanol solution (10% AA solution) as an electrolytic solution, (c) suction filtering the solution obtained by anodic dissolution using a microfilter with a pore size of 0.1 µm, and (d) dividing a mass of electrolytic extraction residue deposited on the microfilter by a difference in mass of the test material before and after the electrolytic extraction.

The higher the content of the M₂₃C₆-type carbide is, the higher the wear resistance is obtained. In order to obtain such an effect, the content of the M₂₃C₆-type carbide is preferably 0.3 mass% or more. The content is more preferably 0.5 mass% or more.

On the other hand, in the case where the content of the M₂₃C₆-type carbide becomes excessive, the hot workability may deteriorate.
Therefore, the content of the M₂₃C₆-type carbide is preferably 3.5 mass% or less. The content is more preferably 3.0 mass% or less.

### 1.2.3. Massive α-Cr Phase

### A. Overview

The "massive α-Cr phase" means an α-Cr phase precipitated at grain boundaries of the y phase. The massive α-Cr phase is different from the fine plate-like α-Cr phase contained in the lamellar structure formed by the aging treatment. The massive α-Cr phase essentially includes Cr.

### B. Average Circle Equivalent Particle Diameter

A "circle equivalent particle diameter of the massive α-Cr phase" refers to a diameter of a circle having an area equal to a cross-sectional area of the massive α-Cr phase in the case where a cross section of the Ni-based alloy is observed with a microscope (SEM-EBSD).

An "average circle equivalent particle diameter of the massive α-Cr phase" is a value calculated using the SEM-EBSD image (phase map) used to calculate the above-mentioned "average circle equivalent particle diameter of the M₂₃C₆-type carbide", and refers to an average value of circle equivalent particle diameters measured for all massive α-Cr phases contained in a freely selected 60 µm × 60 µm region.

The Ni-based alloy before the solution heat treatment includes various massive α-Cr phases with different circle equivalent particle diameters. Among these phases, a fine massive α-Cr phase has an effect of preventing coarsening of the y phase during the solution heat treatment. On the other hand, a coarse massive α-Cr phase is less effective in preventing the coarsening of the y phase, and may rather deteriorate the hot workability.

Note that the M₂₃C₆-type carbide having a circle equivalent particle diameter of 1.0 µm or more has a large particle diameter and thus hardly contribute to the refinement of the y phase.

In order to prevent coarsening of the y phase, it is necessary that the average circle equivalent particle diameter of the massive α-Cr phase is 10.0 µm or less. The average circle equivalent particle diameter is preferably 5.0 µm or less, and more preferably 1.0 µm or less.

### C. Content

A "content of the massive α-Cr phase" is a value calculated using the SEM-EBSD image (phase map) used to calculate the above-mentioned "average circle equivalent particle diameter of the M₂₃C₆-type carbide", and refers to a ratio (area ratio) of a total area of the massive α-Cr phase to an area of a freely selected 60 µm × 60 µm region.

During the solution heat treatment, the larger the content of the massive α-Cr phase, the easier it is to prevent the coarsening of the y phase. In order to obtain such an effect, it is necessary to perform the solution heat treatment so that the massive α-Cr phase remains even after the solution heat treatment. The content of the massive α-Cr phase after the solution heat treatment is preferably 2.0 area% or more. The content is more preferably 3.0 area% or more.

On the other hand, in the case where the content of the massive α-Cr phase is excessive, it may be difficult to form a lamellar structure during the subsequent aging treatment. Therefore, the content of the massive α-Cr phase after the solution heat treatment is preferably 12.0 area% or less. The content is more preferably 10.0 area% or less.

### 1.2.4. Example of Microstructure

FIG. 1 shows an example of a phase map obtained by SEM-EBSD of a Ni-based alloy (Example 4) after the solution heat treatment. In FIG. 1, white particles are the massive α-Cr phase, and gray particles are the y phase. In the case of FIG. 1, the average circle equivalent particle diameter of the massive α-Cr phase was 0.7 µm, and the area ratio thereof was 5.4 area%.

Note that in FIG. 1, no M₂₃C₆-type carbide was observed, but this is because a region without the M₂₃C₆-type carbide was selected and a picture of the structure was taken. In other regions, the M₂₃C₆-type carbide was observed.

### 2. Ni-based Alloy Member (1)

A Ni-based alloy member according to the first embodiment of the present invention is composed of the Ni-based alloy according to the first embodiment of the present invention.

A shape of the Ni-based alloy member is not particularly limited, and an optimum shape can be selected according to a purpose thereof. Examples of the Ni-based alloy member include shaped materials, round bars, and wires. Note that the "shaped material" is a material that is processed into a shape close to the shape of the member or into the shape of the member by hot forging. A member (product) is obtained by finishing the shaped material. Finishing refers to machining and/or heat treatment.

### 3. Ni-based Alloy (2)

### 3.1. Component

The Ni-based alloy according to the second embodiment of the present invention consists of the predetermined elements, with the balance being Ni and unavoidable impurities. The types of additive elements, component ranges thereof, and details of reasons for limitations thereof are the same as in the first embodiment, and therefore, descriptions thereof will be omitted.

### 3.2. Microstructure

### 3.2.1. Cellular Structure

The "cellular structure" refers to a structure in which a lamellar structure of the α-Cr phase and a y phase (y/y' phase) in which a y' phase (Ni₃Al) is precipitated is formed in a state of cell on an entire inside of an austenite phase.

In order to obtain a high strength, it is preferable that the cellular structure is precipitated on the entire inside of the austenite phase.

The Ni-based alloy after the solution heat treatment includes the austenite (initial γ) phase, the M₂₃C₆-type carbide, and the massive α-Cr phase. When the Ni-based alloy after the solution heat treatment is subjected to the aging treatment, the lamellar structure of the α-Cr phase and the y/y' phase is formed in the cell state from the grain boundary to the inside of the grain of the initial y phase, resulting in the cellular structure.

The longer the aging treatment time, the more the cellular structure grows, and eventually the entire of the initial y phase becomes a cellular structure. The cellular structure contributes to increasing the strength of the Ni-based alloy.

### 3.2.2. M₂₃C₆-type Carbide

### A. Overview

The Ni-based alloy according to the present embodiment is obtained by subjecting the Ni-based alloy containing the M₂₃C₆-type carbide after the solution heat treatment (Ni-based alloy according to the first embodiment) to the aging treatment. The circle equivalent particle diameter and content of the M₂₃C₆-type carbide hardly change before and after the aging treatment. Therefore, the Ni-based alloy according to the present embodiment also contains the M₂₃C₆-type carbide. Other points regarding the M₂₃C₆-type carbide are as described above, and therefore, descriptions are omitted.

### B. Average Circle Equivalent Particle Diameter

The definitions of the "circle equivalent particle diameter of the M₂₃C₆-type carbide" and the "average circle equivalent particle diameter of the M₂₃C₆-type carbide" are the same as those in the first embodiment, and therefore, the description thereof will be omitted.

As described above, the larger the average circle equivalent particle diameter of the M₂₃C₆-type carbide is, the higher the wear resistance is obtained. In order to obtain such an effect, it is necessary that the average circle equivalent particle diameter of the M₂₃C₆-type carbide is 1.0 µm or more. The average circle equivalent particle diameter is preferably 2.0 µm or more, and more preferably 5.0 µm or more.

The upper limit of the average circle equivalent particle diameter of the M₂₃C₆-type carbide is not particularly limited, but the average circle equivalent particle diameter is usually 100 µm or less.

### C. Content

The definition of the "content of the M₂₃C₆-type carbide" is the same as in the first embodiment, and therefore, the description thereof is omitted.

As described above, the higher the content of the M₂₃C₆-type carbide is, the higher the wear resistance is obtained. In order to obtain such an effect, the content of the M₂₃C₆-type carbide is preferably 0.3 mass% or more. The content is more preferably 0.5 mass% or more.

### 3.2.3. Massive α-Cr Phase

### A. Overview

The Ni-based alloy according to the present embodiment is obtained by subjecting the Ni-based alloy containing the massive α-Cr phase after the solution heat treatment (Ni-based alloy according to the first embodiment) to the aging treatment.

The circle equivalent particle diameter and content of the massive α-Cr phase hardly change before and after the aging treatment. Therefore, the Ni-based alloy according to the present embodiment also contains the massive α-Cr phase. Other points regarding the massive α-Cr phase are as described above, and therefore, descriptions are omitted.

### B. Average Circle Equivalent Particle Diameter

The definitions of the "circle equivalent particle diameter of the massive α-Cr phase" and the "average circle equivalent particle diameter of the massive α-Cr phase" are the same as those in the first embodiment, and therefore, the description thereof will be omitted.

The size of the massive α-Cr phase contained in the Ni-based alloy before the aging treatment affects the refinement of the y phase, but the size of the massive α-Cr phase contained in the Ni-based alloy after the aging treatment does not significantly affect properties of the Ni-based alloy after the aging treatment.

Since the size of the massive α-Cr phase hardly changes before and after the aging treatment, in the case where the average circle equivalent particle diameter of the massive α-Cr phase after the solution heat treatment is 10.0 µm or less, the average circle equivalent particle diameter of the massive α-Cr phase after the aging treatment is also 10.0 µm or less.

### C. Content

The definition of the "content of the massive α-Cr phase" is the same as in the first embodiment, and therefore, the description thereof is omitted.

The content of the massive α-Cr phase contained in the Ni-based alloy before the aging treatment affects the refinement of the y phase, but the content of the massive α-Cr phase contained in the Ni-based alloy after the aging treatment does not significantly affect properties of the Ni-based alloy after the aging treatment.

Since the content of the massive α-Cr phase hardly changes before and after the aging treatment, in the case where the content of the massive α-Cr phase after the solution heat treatment is 2.0 area% to 12.0 area%, the content of the massive α-Cr phase after the aging treatment is also 2.0 area% to 12.0 area%.

### 3.2.4. Example of Microstructure

FIG. 2 shows an example of a phase map obtained by SEM-EBSD of the Ni-based alloy (Example 4) after the aging treatment. In FIG. 2, black particles are the M₂₃C₆-type carbide, and white particles are the massive α-Cr phase, and gray particles are the cellular structure.

Although it cannot be determined in FIG. 2, the cellular structure is a structure in which the lamellar structure of the α-Cr phase with a thickness of several tens of nm and the y/y' phase is formed in a cell state.

### 3.3. Properties

### 3.3.1. 0.2% Proof Stress

The "0.2% proof stress" refers to a value measured in accordance with JIS Z 2241:2011.

The Ni-based alloy according to the present embodiment includes the cellular structure, and thus exhibits a high 0.2% proof stress. By optimizing manufacturing conditions, the 0.2% proof stress at 25°C becomes 1300 MPa or more. By further optimizing the manufacturing conditions, the 0.2% proof stress at 25°C becomes 1500 MPa or more.

### 3.3.2. Absorption Energy

The "absorption energy" refers to a value measured in accordance with JIS Z 2242:2018.

The Ni-based alloy according to the present embodiment includes the fine cellular structure, and thus exhibits high toughness.
By optimizing the manufacturing conditions, the absorption energy at 25°C becomes 40 J (10R notch) or more. By further optimizing the manufacturing conditions, the absorption energy at 25°C becomes 50 J (10R notch) or more.

### 4. Ni-based Alloy Member (2)

A Ni-based alloy member according to the second embodiment of the present invention is composed of the Ni-based alloy according to the second embodiment of the present invention.

A shape of the Ni-based alloy member is not particularly limited, and an optimum shape can be selected according to a purpose thereof. Examples of the Ni-based alloy member include shaped materials, round bars, and wires.

### 5. Method for Manufacturing Ni-based Alloy

A method for manufacturing the Ni-based alloy according to the present invention includes: (a) a first step of obtaining an ingot by melting and casting a raw material blended to have a predetermined composition, (b) a second step of obtaining a primary hot-worked product by subjecting the ingot to the primary hot working, as necessary, (c) a third step of obtaining a homogenized heat-treated product by subjecting the ingot or the primary hot-worked product to the homogenization heat treatment, as necessary, (d) a fourth step of obtaining a secondary hot-worked product by subjecting the ingot, the primary hot-worked product, or the homogenized heat-treated product to secondary hot working, and (e) a fifth step of obtaining the Ni-based alloy according to the first embodiment of the present invention by subjecting the secondary hot-worked product to the solution heat treatment, wherein the solution heat treatment includes holding the secondary hot-worked product at a temperature in the range of 980°C to 1080°C for at least 0.5 to 1 hour.

The method for manufacturing the Ni-based alloy according to the present invention may further include: (f) a sixth step of obtaining a rough-worked product by roughing the Ni-based alloy (solution-heat-treated product) after the solution heat treatment, and (g) a seventh step of obtaining the Ni-based alloy according to the second embodiment of the present invention by subjecting the rough-worked product or the solution-heat-treated product to the aging treatment.

### 5.1. First Step

First, the raw material blended to have a predetermined composition is melted and cast to obtain the ingot (first step).

The method and conditions for melting and casting are not particularly limited, but the melting is preferably vacuum melting using a vacuum induction furnace. The larger a mold size during casting, the more likely non-uniform distribution of the crystallized carbide occurs due to a non-uniform cooling rate. Therefore, the ingot may be subjected to secondary melting such as electro slag remelting (ESR).

After the secondary melting is applied, an ingot in which the crystallized carbide is uniformly distributed is obtained.

### 5.2. Second Step

Next, if necessary, the ingot is subjected to the primary hot working to obtain the primary hot-worked product (second step).

The "primary hot working" refers to blooming rolling or blooming forging. A temperature of the primary hot working is preferably 900°C to 1150°C.

The primary hot working can be omitted. However, after the ingot is subjected to the primary hot working, casting defects in the ingot can be eliminated and a coarse cast solidified structure can be destroyed. The ingot can be made into a predetermined shape such as a slab, bloom, or billet.

### 5.3. Third Step

Next, if necessary, the ingot or the primary hot-worked product is subjected to the homogenization heat treatment to obtain the homogenized heat-treated product (third step).

A temperature of the homogenization heat treatment is preferably 1200°C to 1280°C. A treatment time is preferably 12 hours or more.

The homogenization heat treatment can be omitted. However, after the ingot or the primary hot-worked product is subjected to the homogenization heat treatment, segregation of components can be mitigated.

### 5.4. Fourth Step

Next, the ingot, the primary hot-worked product, or the homogenized heat-treated product is subjected to the secondary hot working to obtain the secondary hot-worked product (fourth step).

The secondary hot working is performed to form the ingot, the primary hot-worked product, or the homogenized heat-treated product into a predetermined shape (for example, a plate, a bar, a wire rod, or a shaped material). A method for the secondary hot working is not particularly limited, and an optimum method can be selected according to a purpose thereof. Examples of the method for the secondary hot working include hot rolling and hot forging.

The secondary hot working is preferably performed in a temperature range of 900°C to 1200°C. This is because in the case where the temperature of the secondary hot working is too high or too low, cracks are likely to occur during working.

### 5.5. Fifth Step

Next, the secondary hot-worked product is subjected to the solution heat treatment (fifth step). As a result, the Ni-based alloy according to the first embodiment of the present invention is obtained.

After forming into a material having a predetermined shape by the secondary hot working, the material is subjected to the solution heat treatment. In this case, it is important not to allow the massive α-Cr phase to dissolve completely during the solution heat treatment, and intentionally leave a small amount of the fine massive α-Cr phase. In this way, the structure is refined, and the toughness can be ensured.

In the case where a temperature for the solution heat treatment is too low, the amount of the massive α-Cr phase becomes excessive, making it difficult to form the cellular structure during the subsequent aging treatment. Therefore, the temperature for the solution heat treatment is 980°C or higher.

On the other hand, in the case where the temperature for the solution heat treatment is too high, the massive α-Cr phase is completely dissolved and crystal grains are coarsened. As a result, the toughness of the Ni-based alloy is lowered. Therefore, the temperature for the solution heat treatment is 1080°C or lower.

A time of approximately 0.5 hours to 1 hour is sufficient for the solution heat treatment.

After holding for a predetermined time at the solution heat treatment temperature, the material is quenched. In this case, in the case where a cooling rate is too slow, there is concern that the cellular structure may be partially formed during cooling. Cracking may occur in the case where the cellular structure is partially formed during cooling. The hardness may also increase, and roughing such as cutting may become difficult. Therefore, as for the cooling method, it is preferable to use a technique that provides a cooling rate higher than that of oil cooling. The faster the cooling rate, the better.

### 5.6. Sixth Step

Next, if necessary, the solution-heat-treated product is subjected to roughing to obtain the rough-worked product (sixth step).

The roughing is performed as necessary. A roughing method is not particularly limited, and an optimum method can be selected according to a purpose thereof. Examples of the roughing method include cutting and cold working.

### 5.7. Seventh Step

Next, the rough-worked product or the solution-heat-treated product is subjected to the aging treatment (seventh step). As a result, the Ni-based alloy according to the second embodiment of the present invention is obtained.

The aging treatment is performed to form a cellular structure of a lamellar structure of the α-Cr phase and the y/y' phase inside the y phase, which is a matrix phase. A temperature for the aging treatment is usually 500°C to 800°C. A time for the aging treatment is usually 1 hour to 50 hours. Cooling after the aging treatment may be air cooling.

Since the strength the Ni-based alloy and the toughness (impact property) thereof are in a trade-off relation, it is preferable to set the aging treatment conditions in consideration of the target strength and toughness.

For example, in the case where a Ni-based alloy having a 0.2% proof stress of 1300 MPa or more and an impact property of 50 J (10R notch) or more, with an emphasis on toughness, is desired, it is preferable to set the aging treatment temperature to 710°C to 750°C and the aging treatment time to approximately 16 hours.

Alternatively, in the case where a Ni-based alloy having a 0.2% proof stress of 1500 MPa or more and an impact property of 40 J (10R notch) or more, with an emphasis on strength, is desired, it is preferable to set the aging treatment temperature to 600°C to 700°C and the aging treatment time to approximately 16 hours.

### 6. Effects

In the case where the raw material of the Ni-based alloy containing a relatively large amount of C is melted and cast, an ingot containing the massive α-Cr phase and crystallized coarse M₂₃C₆-type carbide particles can be obtained. If necessary, the obtained ingot is subjected to the primary hot working, homogenization heat treatment, and secondary hot working, and then solution heat treatment at a relatively low temperature, so that a fine massive α-Cr phase remains without being dissolved. As a result, the fine massive α-Cr phase functions as pinning particles, and during the solution heat treatment, coarsening of the y phase can be prevented. Furthermore, when the aging treatment is applied to the Ni-based alloy after the solution heat treatment, the cellular structure is formed on the entire inside of the y phase.

The Ni-based alloy according to the present invention is excellent in corrosion resistance and hot workability due to an optimized composition thereof. The Ni-based alloy after the aging treatment exhibits high wear resistance since the coarse M₂₃C₆-type carbide particles are dispersed in a matrix. Furthermore, the Ni-based alloy after the aging treatment exhibits high strength due to the inclusion of the cellular structure. Since an initial y phase is fine, the cellular structure is also fine, and high toughness (that is, high impact resistance) is also exhibited.

### EXAMPLES

### Examples 1 to 10, Comparative Examples 1 to 7

### 1. Preparation of Samples

In a vacuum induction furnace, 50 kg of a raw material having a composition shown in Table 1 was vacuum melted to obtain an ingot. The obtained ingot was subjected to the homogenization heat treatment at 1200°C for 24 hours, and then hot forging in a temperature range of 900°C to 1200°C to produce a round bar with a diameter of 24 mm. The round bar was subjected to the solution heat treatment at 1050°C for 1 hour, and then cooled with water. The round bar was further subjected to the aging treatment at 720°C for 16 hours and then air-cooled.

**Table 1**

| | Composition (mass%) | | | | | | | | | |
|---|---|---|---|---|---|---|---|---|---|---|
| | C | Si | Mn | P | S | Cu | Ni | Cr | Mo | Al |
| Example 1 | 0.14 | 0.07 | 0.01 | 0.004 | 0.0010 | < 0.05 | Bal. | **36.2** | < 0.1 | 3.3 |
| Example 2 | 0.18 | 0.10 | 0.01 | 0.003 | 0.0012 | < 0.05 | Bal. | **36.5** | 1.5 | 4.5 |
| Example 3 | 0.19 | 0.09 | 0.02 | 0.006 | 0.0009 | **2.1** | Bal. | **38.2** | < 0.1 | 4.0 |
| Example 4 | 0.15 | 0.08 | 0.01 | 0.005 | 0.0015 | < 0.05 | Bal. | **36.2** | < 0.1 | 3.8 |
| Example 5 | 0.22 | 0.05 | 0.03 | 0.006 | 0.0006 | < 0.05 | Bal. | **38.0** | < 0.1 | 3.9 |
| Example 6 | 0.24 | 0.09 | 0.02 | 0.002 | 0.0011 | < 0.05 | Bal. | **38.4** | < 0.1 | 3.7 |
| Example 7 | 0.20 | 0.06 | 0.01 | 0.004 | 0.0007 | < 0.05 | Bal. | **35.8** | < 0.1 | 3.6 |
| Example 8 | 0.15 | 0.07 | 0.01 | 0003 | 0.0008 | < 0.05 | Bal. | **37.4** | < 0.1 | 3.4 |
| Example 9 | 0.26 | 0.07 | 0.02 | 0.004 | 0.0010 | < 0.05 | Bal. | **36.5** | < 0.1 | 3.6 |
| Example 10 | 0.19 | 0.10 | 0.01 | 0.005 | 0.0011 | < 0.05 | Bal. | **37.6** | < 0.1 | 4.0 |
| Comparative Example 1 | 3.00 | 0.09 | 0.01 | 0.002 | 0.0011 | < 0.05 | Bal. | **40.0** | < 0.1 | **6.0** |
| Comparative Example 2 | 0.31 | 0.05 | 0.01 | 0.003 | 0.0009 | < 0.05 | Bal. | **37.6** | < 0.1 | **3.8** |
| Comparative Example 3 | 0.31 | 0.05 | 0.01 | 0.003 | 0.0009 | <0.05 | Bal. | **37.6** | < 0.1 | **3.8** |
| Comparative Example 4 | 0.23 | 0.09 | 0.01 | 0.005 | 0.0012 | < 0.05 | Bal. | **29.3** | < 0.1 | **4.0** |
| Comparative Example 5 | 0.19 | 0.06 | 0.01 | 0.003 | 0.0007 | < 0.05 | Bal. | **43.3** | < 0.1 | **3.5** |
| Comparative Example 6 | 0.07 | 0.09 | 0.01 | 0.004 | 0.0008 | < 0.05 | Bal. | **37.8** | < 0.1 | **3.7** |
| Comparative Example 7 | 0.15 | 0.09 | 0.01 | 0.005 | 0.0015 | < 0.05 | Bal. | **36.2** | < 0.1 | **3.8** |

**Table 1 (continued)**

| | Composition (mass%) | | | | | | | | |
|---|---|---|---|---|---|---|---|---|---|
| | Nb | Ti | v | Fe | B | Mg | Ca | O | N |
| Example 1 | < 0.05 | < 0.05 | < 0.05 | < 1.0 | 0.0032 | 0.0021 | - | < 0.0020 | < 0.0200 |
| Example 2 | < 0.05 | < 0.05 | < 0.05 | < 1.0 | 0.0035 | - | 0.0024 | < 0.0020 | < 0.0200 |
| Example 3 | < 0.05 | < 0.05 | < 0.05 | < 1.0 | 0.0033 | 0.0019 | - | < 0.0020 | < 0.0200 |
| Example 4 | < 0.05 | < 0.05 | < 0.05 | < 1.0 | 0.0030 | 0.0034 | - | < 0.0020 | < 0.0200 |
| Example 5 | < 0.05 | < 0.05 | < 0.05 | < 1.0 | 0.0028 | 0.0020 | - | < 0.0020 | < 0.0200 |
| Example 6 | < 0.05 | < 0.05 | < 0.05 | < 1.0 | 0.0036 | 0.0028 | - | < 0.0020 | < 0.0200 |
| Example 7 | < 0.05 | < 0.05 | < 0.05 | < 1.0 | 0.0031 | - | 0.0036 | < 0.0020 | < 0.0200 |
| Example 8 | < 0.05 | < 0.05 | < 0.05 | < 1.0 | 0.0034 | - | - | < 0.0020 | < 0.0200 |
| Example 9 | < 0.05 | < 0.05 | < 0.05 | < 1.0 | 0.0029 | 0.0027 | 0.0022 | < 0.0020 | < 0.0200 |
| Example 10 | < 0.05 | < 0.05 | < 0.05 | < 1.0 | - | 0.0018 | 0.0027 | < 0.0020 | < 0.0200 |
| Comparative Example 1 | < 0.05 | < 0.05 | < 0.05 | < 1.0 | 0.0028 | | - | < 0.0020 | < 0.0200 |
| Comparative Example 2 | < 0.05 | < 0.05 | 1.43 | < 1.0 | 0.0033 | | - | < 0.0020 | < 0.0200 |
| Comparative Example 3 | < 0.05 | < 0.05 | 1.43 | < 1.0 | 0.0033 | | - | < 0.0020 | < 0.0200 |
| Comparative Example 4 | < 0.05 | < 0.05 | < 0.05 | < 1.0 | 0.0036 | | - | < 0.0020 | < 0.0200 |
| Comparative Example 5 | < 0.05 | < 0.05 | < 0.05 | < 1.0 | 0.0029 | | - | < 0.0020 | < 0.0200 |
| Comparative Example 6 | < 0.05 | < 0.05 | < 0.05 | < 1.0 | 0.0030 | | - | < 0.0020 | < 0.0200 |
| Comparative Example 7 | < 0.05 | < 0.05 | < 0.05 | < 1.0 | 0.0030 | 0.0034 | - | < 0.0020 | < 0.0200 |

### 2. Test Method

### 2.1. Average Grain Diameter of y Phase After Solution Heat Treatment

Using the line segment method, the average grain diameter of the y phase contained in the Ni-based alloy after the solution heat treatment was measured. First, a photograph of a metal structure of the round bar was captured with an optical microscope (magnification: 100 times).
Next, a total of ten different straight lines of five vertical lines and five horizontal lines were drawn on the captured photograph, and for each of the straight lines, a value (= L/n) obtained by dividing a length (L) of the straight line by the number (n) of crystal grains whose boundaries intersect with the straight line was calculated. Further, an average grain diameter was calculated by calculating an average value thereof.

### 2.2. Weight Fraction of M₂₃C₆-type Carbide

Using an electrolytic extraction method, a weight fraction of the M₂₃C₆-type carbide contained in the Ni-based alloy after the aging treatment was measured.

### 2.3. 0.2% Proof Stress and Elongation

A tensile test was performed at room temperature in accordance with JIS Z 2241:2011 to measure 0.2% proof stress and elongation.

### 2.4. Absorption Energy

A Charpy impact test (notch R: 10 mm) was performed in accordance with JIS Z 2242:2018 to measure absorption energy.

### 2.5. Wear Resistance

The wear resistance was evaluated in accordance with ASTM G65 Procedure A. A weight change (g) of a wheel before and after the test was measured with a test load of 30 Lbf (13.608 kg), a sand flow rate of 320 g/min, a wheel diameter of 8.68" (220.472 mm), and a wheel width of 0.5" (12.7 mm).

### 3. Results

Table 2 shows results. The followings can be found from Table 2.
(1) Comparative Example 1 corresponds to the Ni-based alloy disclosed in JP4981212B2. In Comparative Example 1, a large amount of the M₂₃C₆-type carbide precipitated due to the excessive amount of C. As a result, hot working became difficult, and various evaluations could not be performed.
(2) Comparative Examples 2 and 3 correspond to the Ni-based alloy disclosed in Patent Literature 2.

Comparative Example 2 has a high 0.2% proof stress, but a small elongation and a small absorption energy. It is considered that this is because the amount of C is excessive and V is contained.

Compared with Comparative Example 2, Comparative Example 3 had smaller elongation and absorption energy. It is considered that this is because the solution heat treatment temperature was too high, and the average grain diameter of the y phase after the solution heat treatment exceeded 50 µm.

(3) Comparative Example 4 has a low 0.2% proof stress and poor wear resistance. It is considered that this is because the amount of Cr is small.

(4) In Comparative Example 5, since the amount of Cr was excessive, a large amount of the massive α-Cr phase with poor deformability was precipitated. As a result, hot working became difficult, and various evaluations could not be performed.

(5) Comparative Example 6 had a high 0.2% proof stress and a large absorption energy, but the wear resistance thereof was lowered. It is considered that this is because the amount of C is small.

(6) Comparative Example 7 has a small absorption energy. It is considered that this is because the solution heat treatment temperature was too high, and the average grain diameter of the y phase after the solution heat treatment exceeded 50 µm.

(7) All of Examples 1 to 10 had a 0.2% proof stress of 1400 MPa or more and an absorption energy of 50 J or more. All weight changes after the wear resistance test were less than 2 g.

(8) For each sample after the solution heat treatment and after the aging treatment, the average circle equivalent particle diameter of the massive α-Cr phase and the area ratio of the massive α-Cr phase were calculated using SEM-EBSD. As a result, in each of Examples 1 to 10, the average circle equivalent particle diameter of the massive α-Cr phase after the solution heat treatment and after the aging treatment was 10.0 µm or less. In each of Examples 1 to 10, the area ratio of the massive α-Cr phase after the solution heat treatment and after the aging treatment was in the range of 2.0 area% to 12.0 area%.

(9) For each sample after the solution heat treatment and after the aging treatment, the average circle equivalent particle diameter of the M₂₃C₆-type carbide was calculated using SEM-EBSD. As a result, in each of Examples 1 to 10, the average circle equivalent particle diameter of the M₂₃C₆-type carbide after the solution heat treatment and after the aging treatment was 1.0 µm or more.

**Table 2**

| | **Conditions for solution heat treatment** | **Grain diameter [µm] after solution heat treatment** | Carbide weight fraction [%] |
|---|---|---|---|
| Example 1 | **1050°C, 1h, water cooling** | 17 | 1.1 |
| Example 2 | **1050°C, 1h, water cooling** | 16 | 1.7 |
| Example 3 | **1050°C, 1h, water cooling** | 10 | 1.8 |
| Example 4 | **1050°C, 1h, water cooling** | 7 | 1.3 |
| Example 5 | **1050°C, 1h, water cooling** | 6 | 2.1 |
| Example 6 | **1050°C, 1h, water cooling** | 14 | 2.3 |
| Example 7 | **1050°C, 1h, water cooling** | 11 | 1.8 |
| Example 8 | **1050°C, 1h, water cooling** | 16 | 1.2 |
| Example 9 | **1050°C, 1h, water cooling** | 15 | 2.4 |
| Example 10 | **1050°C, 1h, water cooling** | 18 | 1.6 |
| Comparative Example 1 | - | - | - |
| Comparative Example 2 | **1050°C, 1h, water cooling** | 11 | 3.0 |
| Comparative Example 3 | **1150°C, 1h, water cooling** | 290 | 3.0 |
| Comparative Example 4 | **1050°C, 1h, water cooling** | 47 | 2.1 |
| Comparative Example 5 | - | - | - |
| Comparative Example 6 | **1150°C, 1h, water cooling** | 310 | - |
| Comparative Example 7 | **1150°C, 1h, water cooling** | 330 | 1.3 |

**Table 2 (continued)**

| | 0.2% Proof stress [Mpa] | Elongation [%] | Absorption energy [J] | Wear resistance (weight change [g]) |
|---|---|---|---|---|
| Example 1 | 1501 | 6.5 | 101 | 1.71 |
| Example 2 | 1470 | 8.0 | 134 | 1.47 |
| Example 3 | 1492 | 6.3 | 99 | 1.54 |
| Example 4 | 1477 | 8.1 | 136 | 2.01 |
| Example 5 | 1522 | 5.6 | 91 | 1.59 |
| Example 6 | 1537 | 7.9 | 127 | 1.62 |
| Example 7 | 1530 | 6.9 | 115 | 1.93 |
| Example 8 | 1480 | 7.1 | 114 | 1.57 |
| Example 9 | 1541 | 5.4 | 89 | 1.56 |
| Example 10 | 1496 | 8.7 | 149 | 1.54 |
| Comparative Example 1 | Unevaluated due to poor hot workability | | | |
| Comparative Example 2 | 1593 | 2.4 | 25 | 1.55 |
| Comparative Example 3 | 1542 | 0.9 | 8 | 1.63 |
| Comparative Example 4 | 1125 | 14.7 | 178 | 2.89 |
| Comparative Example 5 | Unevaluated due to poor hot workability | | | |
| Comparative Example 6 | 1489 | 9.9 | 156 | 2.63 |
| Comparative Example 7 | 1576 | 2.9 | 29 | 1.66 |

Although the embodiment of the present invention has been described in detail above, the present invention is not limited to the above embodiment, and various modifications can be made without departing from the scope of the appended claims.

The present application is based on Japanese Patent Applications No. 2022-174050 filed on October 31, 2022 and No. 2023-128787 filed on August 7, 2023.

### INDUSTRIAL APPLICABILITY

The Ni-based alloy according to the present invention can be used for members for oil and gas drilling, various shaped materials including a shaped material for members for oil and gas drilling, round bars, wires, and the like.

## Claims

1. A Ni-based alloy consisting of: $0.10 mass % < C \leq 0.30 mass % ;$ $Si \leq 0.50 mass % ;$ $Mn \leq 0.50 mass % ;$ $P \leq 0.030 mass % ;$ $S \leq 0.010 mass % ;$ $Cu \leq 3.00 mass % ;$ $30.0 mass % \leq Cr \leq 39.0 mass % ;$ $Mo \leq 3.00 mass % ;$ $Fe \leq 3.00 mass % ;$ $2.00 mass % \leq Al \leq 5.00 mass % ;$ $O \leq 0.0100 mass % ;$ $N \leq 0.050 mass % ;$ $Nb \leq 0.50 mass % ;$ $V \leq 0.50 mass % ;$ $Ti \leq 0.50 mass % ;$ $Ta \leq 0.50 mass ;$ $W \leq 0.50 mass % ;$ and
at least one element selected from the group consisting of 0.0010 mass% ≤ B ≤ 0.0100 mass%, 0.0010 mass% ≤ Mg ≤ 0.0100 mass%, and 0.0010 mass% ≤ Ca ≤ 0.0100 mass%,
with the balance being Ni and unavoidable impurities, wherein
the Ni-based alloy comprises
an austenite phase (y phase) having an average grain diameter of 50.0 µm or less,
a M₂₃C₆-type carbide having an average circle equivalent particle diameter of 1.0 µm or more, and
a massive α-Cr phase, precipitated at grain boundaries of the y phase, having an average circle equivalent particle diameter of 10.0 µm or less, wherein the average grain diameter of the y phase, the average circle equivalent particle diameter of the M₂₃C₆-type carbide and the average circle equivalent particle diameter of the massive α-Cr phase are measured as set out in the description.

2. A Ni-based alloy member comprising the Ni-based alloy according to claim 1.

3. A Ni-based alloy consisting of: $0.10 mass % < C \leq 0.30 mass % ;$ $Si \leq 0.50 mass % ;$ $Mn \leq 0.50 mass % ;$ $P \leq 0.030 mass % ;$ $S \leq 0.010 mass % ;$ $Cu \leq 3.00 mass % ;$ $30.0 mass % \leq Cr \leq 39.0 mass % ;$ $Mo \leq 3.00 mass % ;$ $Fe \leq 3.00 mass % ;$ $2.00 mass % \leq Al \leq 5.00 mass % ;$ $O \leq 0.0100 mass % ;$ $N \leq 0.050 mass % ;$ $Nb \leq 0.50 mass % ;$ $V \leq 0.50 mass % ;$ $Ti \leq 0.50 mass % ;$ $Ta \leq 0.50 mass ;$ $W \leq 0.50 mass % ;$ and
at least one element selected from the group consisting of 0.0010 mass% ≤ B ≤ 0.0100 mass%, 0.0010 mass% ≤ Mg ≤ 0.0100 mass%, and 0.0010 mass% ≤ Ca ≤ 0.0100 mass%,
with the balance being Ni and unavoidable impurities, wherein
the Ni-based alloy comprises
a cellular structure,
a M₂₃C₆-type carbide having an average circle equivalent particle diameter of 1.0 µm or more, and
a massive α-Cr phase having an average circle equivalent particle diameter of 10.0 µm or less,
wherein the cellular structure is a structure in which a lamellar structure of the α-Cr phase and a y phase in which a y' phase is precipitated is formed in a state of cell on an entire inside of an austenite phase,
wherein the Ni-based alloy has a 0.2% proof stress at 25°C of 1300 MPa or more, and
wherein the Ni-based alloy has an absorption energy at 25°C of 40 J (10 R notch) or more,
wherein the 0.2% proof stress, the absorption energy, the average circle equivalent particle diameter of the M₂₃C₆-type carbide and the average circle equivalent particle diameter of the massive α-Cr phase are measured as set out in the description.

4. A Ni-based alloy member comprising the Ni-based alloy according to claim 3.

5. A method for manufacturing a Ni-based alloy, the method comprising:
a first step of obtaining an ingot by melting and casting a raw material blended to have a predetermined composition;
a second step of obtaining a primary hot-worked product by subjecting the ingot to primary hot working;
a third step of obtaining a homogenized heat-treated product by subjecting the primary hot-worked product to homogenization heat treatment;
a fourth step of obtaining a secondary hot-worked product by subjecting the homogenized heat-treated product to secondary hot working; and
a fifth step of obtaining the Ni-based alloy according to claim 1 by subjecting the secondary hot-worked product to solution heat treatment, wherein the solution heat treatment includes holding the secondary hot-worked product at a temperature in the range of 980°C to 1080°C for at least 0.5 to 1 hour.

6. The method for manufacturing a Ni-based alloy according to claim 5, the method further comprising:
a seventh step of obtaining the Ni-based alloy according to claim 3 by subjecting the Ni-based alloy after the solution heat treatment to aging treatment.

7. The method according to claim 5 or 6, further comprising using the Ni-based alloy so manufactured for making members for oil and/or gas drilling.

8. The method according to claim 7, wherein the member so made is a round bar or a wire.

9. Use of the Ni-based alloy according to claim 1 or 3, or the Ni-based alloy member according to claim 2 or 4, for members for oil and/or gas drilling, in particular shaped materials therefor such as round bars or wires.

## Patentansprüche

1. Ni-basierte Legierung aus: $0 , 10 Massen % < C \leq 0 , 30 Massen % ;$ $Si \leq 0,50 Massen % ;$ $Mn \leq 0,50 Massen % ;$ $P \leq 0 , 030 Massen % ;$ $S \leq 0 , 010 Massen % ;$ $Cu \leq 3,00 Massen % ;$ $30 , 0 Massen % \leq Cr \leq 39,0 Massen % ;$ $Mo \leq 3,00 Massen % ;$ $Fe \leq 3,00 Massen % ;$ $2 , 00 Massen % \leq Al \leq 5 , 0 0 Massen % ;$ $O \leq 0,0100 Massen % ;$ $N \leq 0,050 Massen % ;$ $Nb \leq 0,50 Massen % ;$ $V \leq 0,50 Massen % ;$ $Ti \leq 0,50 Massen % ;$ $Ta \leq 0,50 Massen ;$ $W \leq 0,50 Massen % ;$ und
wenigstens einem aus der Gruppe ausgewählten Element, die aus 0,0010 Massen% ≤ B ≤ 0,0100 Massen%, 0,0010 Massen% ≤ Mg ≤ 0,0100 Massen% und 0,0010 Massen% ≤ Ca ≤ 0,0100 Massen% besteht,
mit dem Rest Ni und unvermeidliche Verunreinigungen, wobei die Ni-basierte Legierung umfasst:
ein Austenit-Phase (γ-Phase) mit einem durchschnittlichen Korndurchmesser von 50,0 µm oder weniger,
einem M₂₃C₆-Typ-Carbid mit einem durchschnittlichen Äquivalentkreis-Partikeldurchmesser von 1,0 µm oder mehr, und
einer massiven α-Cr-Phase, ausgeschieden an Korngrenzen der γ-Phase, mit einem durchschnittlichen Äquivalentkreis-Partikeldurchmesser von 10,0 µm oder weniger, wobei der durchschnittliche Korndurchmesser der γ-Phase, der durchschnittliche Äquivalentkreis-Partikeldurchmesser des M₂₃C₆-Typ-Carbids und der durchschnittliche Äquivalentkreis-Partikeldurchmesser der massiven α-Cr-Phase wie in der Beschreibung ausgeführt gemessen werden.

2. Ni-basiertes Legierungsbauteil umfassend die Ni-basierte Legierung gemäß Anspruch 1.

3. Ni-basierte Legierung aus: $0 , 10 Massen % < C \leq 0,30 Massen % ;$ $Si \leq 0 , 50 Massen % ;$ $Mn \leq 0 , 50 Massen % ;$ $P \leq 0,030 Massen % ;$ $S \leq 0 , 010 Massen % ;$ $Cu \leq 3 , 00 Massen % ;$ $30 , 0 Massen % \leq Cr \leq 39 , 0 Massen % ;$ $Mo \leq 3,00 Massen % ;$ $Fe \leq 3 , 00 Massen % ;$ $2 , 00 Massen % \leq Al \leq 5 , 00 Massen % ;$ $O \leq 0 , 0100 Massen % ;$ $N \leq 0,050 Massen % ;$ $Nb \leq 0 , 50 Massen % ;$ $V \leq 0,50 Massen % ;$ $Ti \leq 0,50 Massen % ;$ $Ta \leq 0,50 Massen ;$ $W \leq 0,50 Massen % ;$ und
wenigstens einem aus der Gruppe ausgewählten Element, die aus 0,0010 Massen% ≤ B ≤ 0,0100 Massen%, 0,0010 Massen% ≤ Mg ≤ 0,0100 Massen% und 0,0010 Massen% ≤ Ca ≤ 0,0100 Massen% besteht,
mit dem Rest Ni und unvermeidliche Verunreinigungen, wobei
die Ni-basierte Legierung umfasst
eine Zell-Struktur,
ein M₂₃C₆-Typ-Carbid mit einem durchschnittlichen Äquivalentkreis-Partikeldurchmesser von 1,0 µm oder mehr, und
einer massiven α-Cr-Phase mit einem durchschnittlichen Äquivalentkreis-Partikeldurchmesser von 10,0 µm oder weniger,
wobei die Zell-Struktur eine Struktur ist, bei der eine Lamellen-Struktur der α-Cr-Phase und eine γ-Phase, in welcher eine y'-Phase ausgeschieden ist, im Zustand einer Zelle in einem gesamten Inneren einer Austenit-Phase gebildet ist,
wobei die Ni-basierte Legierung eine 0,2%-Prüfspannung bei 25°C von 1300 MPa oder mehr zeigt, und
wobei die Ni-basierte Legierung eine Absorptions-Energie bei 25°C von 40 J (10 R-Kerbe) oder mehr zeigt,
wobei die 0,2%-Prüfspannung, die Absorptions-Energie, der durchschnittliche Äquivalentkreis-Durchmesser des M₂₃C₆-Typ-Carbids und der durchschnittliche Äquivalentkreis-Durchmesser der massiven α-Cr-Phase wie in der Beschreibung ausgeführt gemessen werden.

4. Ni-basiertes Legierungsbauteil umfassend die Ni-basierte Legierung gemäß Anspruch 3.

5. Verfahren zum Herstellen einer Ni-basierten Legierung, das Verfahren umfassend:
einen ersten Schritt des Erhaltens eines Ingots durch Schmelzen und Gießen eines derart gemischten Rohmaterials, dass er eine vorbestimmte Zusammensetzung aufweist;
einen zweiten Schritt des Erhaltens eines primären warmumgeformten Produkts durch Unterziehen des Ingots einem primären Warmbearbeiten;
einen dritten Schritt des Erhaltens eines homogenisierten wärmebehandelten Produkts durch Unterziehen des primären warmumgeformten Produkts einer Homogenisierungs-Wärmebehandlung;
einen vierten Schritt des Erhaltens eines sekundären warmumgeformten Produkts durch Unterziehen des homogenisierten wärmebehandelten Produkts einem sekundären Warmumformen; und
einen fünften Schritt des Erhaltens der Ni-basierten Legierung gemäß Anspruch 1 durch Unterziehen des sekundären warmumgeformten Produkts einer Lösungs-Wärmebehandlung, wobei die Lösungs-Wärmebehandlung ein Halten des sekundären warmumgeformten Produkts für wenigstens 0,5 bis 1 Stunde bei einer Temperatur im Bereich von 980°C bis 1080°C beinhaltet.

6. Verfahren zum Herstellen einer Ni-basierten Legierung gemäß Anspruch 5, wobei das Verfahren ferner umfasst:
einen siebten Schritt des Erhaltens der Ni-basierten Legierung gemäß Anspruch 3 durch Unterziehen der Ni-basierten Legierung, nach der Lösungs-Wärmebehandlung, einer Auslagerungs-Behandlung.

7. Verfahren gemäß Anspruch 5 oder 6, ferner umfassend Verwenden der so hergestellten Ni-basierten Legierung für Bauteile für das Öl- und/oder Gas-Bohren.

8. Verfahren gemäß Anspruch 7, wobei das so hergestellte Bauteil ein Rundstab oder ein Draht ist.

9. Verwendung der Ni-basierten Legierung gemäß Anspruch 1 oder 3, oder des Ni-basierten Legierungsbauteils gemäß Anspruch 2 oder 4, für Bauteile zum Öl- und/oder Gas-Bohren, insbesondere dafür gestaltete Materialien wie Rundstäbe oder Drähte.

## Revendications

1. Alliage à base de Ni constitué de : $0 , 10 % en masse < C \leq 0 , 30 % en masse ;$ $Si \leq 0 , 50 % en masse ;$ $Mn \leq 0 , 50 % en masse ;$ $P \leq 0,030 % en masse ;$ $S \leq 0,010 % en masse ;$ $Cu \leq 3,00 % en masse ;$ $30 , 0 % en masse \leq Cr \leq 39 , 0 % en masse ;$ $Mo \leq 3 , 00 % en masse ;$ $Fe \leq 3,00 % en masse ;$ $2 , 00 % en masse \leq Al \leq 5 , 00 % en masse ;$ $O \leq 0,0100 % en masse ;$ $N \leq 0,050 % en masse ;$ $Nb \leq 0,50 % en masse ;$ $V \leq 0,50 % en masse ;$ $Ti \leq 0,50 % en masse ;$ $Ta \leq 0,50 % en masse ;$ $W \leq 0 , 50 % en masse ;$ et
au moins un élément choisi dans le groupe constitué de 0,0010 % en masse ≤ B ≤ 0,0100 % en masse, 0,0010 % en masse ≤ Mg ≤ 0,0100 % en masse, et 0,0010 % en masse ≤ Ca ≤ 0,0100 % en masse,
le reste étant Ni et des impuretés inévitables, dans lequel
l'alliage à base de Ni comprend
une phase austénitique (phase γ) ayant un diamètre moyen de grains de 50,0 µm ou moins,
un carbure de type M₂₃C₆ ayant un diamètre de cercle équivalent moyen de particules de 1,0 µm ou plus, et
une phase α-Cr massive, précipitée aux joints de grains de la phase γ, ayant un diamètre de cercle équivalent moyen de particules de 10,0 µm ou moins, dans lequel le diamètre moyen de grains de la phase γ, le diamètre de cercle équivalent moyen de particules du carbure de type M₂₃C₆ et le diamètre de cercle équivalent moyen de particules de la phase α-Cr massive sont mesurés comme indiqué dans la description.

2. Élément en alliage à base de Ni comprenant l'alliage à base de Ni selon la revendication 1.

3. Alliage à base de Ni constitué de : $0 , 10 % en masse < C \leq 0 , 30 % en masse ;$ $Si \leq 0,50 % en masse ;$ $Mn \leq 0,50 % en masse ;$ $P \leq 0,030 % en masse ;$ $S \leq 0,010 % en masse ;$ $Cu \leq 3,0 % en masse ;$ $30,0 % en masse \leq Cr \leq 39,0 % en masse ;$ $Mo \leq 3,00 % en masse ;$ $Fe \leq 3,00 % en masse ;$ $2,00 % en masse \leq Al \leq 5,00 % en masse ;$ $O \leq 0,0100 % en masse ;$ $N \leq 0,050 % en masse ;$ $Nb \leq 0 , 50 % en masse ;$ $V \leq 0 , 50 % en masse ;$ $Ti \leq 0 , 50 % en masse ;$ $Ta \leq 0 , 50 % en masse ;$ $W \leq 0 , 50 % en masse ;$ et
au moins un élément choisi dans le groupe constitué de 0,0010 % en masse ≤ B ≤ 0,0100 % en masse, 0,0010 % en masse ≤ Mg ≤ 0,0100 % en masse, et 0,0010 % en masse ≤ Ca ≤ 0,0100 % en masse,
le reste étant Ni et des impuretés inévitables, dans lequel
l'alliage à base de Ni comprend
une structure cellulaire,
un carbure de type M₂₃C₆ ayant un diamètre de cercle équivalent moyen de particules de 1,0 µm ou plus, et
une phase α-Cr massive ayant un diamètre de cercle équivalent moyen de particules de 10,0 µm ou moins,
dans lequel la structure cellulaire est une structure dans laquelle une structure lamellaire de la phase α-Cr et d'une phase γ dans laquelle une phase γ' est précipitée est formée dans un état de cellule sur l'ensemble d'un intérieur d'une phase austénitique,
dans lequel l'alliage à base de Ni a une limite d'élasticité à 0,2 % à 25 °C de 1 300 MPa ou plus, et
dans lequel l'alliage à base de Ni a une énergie d'absorption à 25 °C de 40 J (encoche de 10 R) ou plus,
dans lequel la contrainte d'élasticité à 0,2 %, l'énergie d'absorption, le diamètre de cercle équivalent moyen de particules du carbure de type M₂₃C₆ et le diamètre de cercle équivalent moyen de particules de la phase α-Cr massive sont mesurés comme indiqué dans la description.

4. Élément en alliage à base de Ni comprenant l'alliage à base de Ni selon la revendication 3.

5. Procédé de fabrication d'un alliage à base de Ni, le procédé comprenant :
une première étape d'obtention d'un lingot par fusion et coulée d'une matière brute mélangée pour obtenir une composition prédéterminée ;
une deuxième étape d'obtention d'un produit primaire travaillé à chaud en soumettant le lingot à un traitement primaire à chaud ;
une troisième étape d'obtention d'un produit traité thermiquement homogénéisé en soumettant le produit primaire travaillé à chaud à un traitement thermique d'homogénéisation ;
une quatrième étape d'obtention d'un produit secondaire travaillé à chaud en soumettant le produit traité thermiquement homogénéisé à un travail à chaud secondaire ; et
une cinquième étape d'obtention de l'alliage à base de Ni selon la revendication 1 en soumettant le produit travaillé à chaud secondaire à un traitement thermique en solution, dans lequel le traitement thermique en solution comporte le maintien du produit travaillé à chaud secondaire à une température comprise dans la plage de 980 °C à 1 080 °C pendant au moins 0,5 à 1 heure.

6. Procédé de fabrication d'un alliage à base de Ni selon la revendication 5, le procédé comprenant en outre :
une septième étape d'obtention de l'alliage à base de Ni selon la revendication 3 en soumettant l'alliage à base de Ni après le traitement thermique en solution à un traitement de vieillissement.

7. Procédé selon la revendication 5 ou 6, comprenant en outre l'utilisation de l'alliage à base de Ni ainsi fabriqué pour fabriquer des éléments de forage pétrolier et/ou gazier.

8. Procédé selon la revendication 7, dans lequel l'élément ainsi fabriqué est une barre ronde ou un fil.

9. Utilisation de l'alliage à base de Ni selon la revendication 1 ou 3, ou de l'élément en alliage à base de Ni selon la revendication 2 ou 4, pour des éléments de forage pétrolier et/ou gazier, en particulier des matériaux façonnés pour ceux-ci, tels que des barres rondes ou des fils.
